

## UNITED STATES PATENT OFFICE

2,455,169

## COLORED COUPLERS

Dudley B. Glass, Paul W. Vittum, and Arnold Weissberger, Rochester, N. Y., assignors to Eastman Kodak Company, Rochester, N. Y., a corporation of New Jersey

No Drawing. Application May 3, 1944,  
Serial No. 533,931

5 Claims. (Cl. 95-6)

1

This invention relates to color photography and particularly to coupler compounds for use in photographic processes.

Color-forming compounds which react with the development product of aromatic amino developing agents to form colored images upon photographic development are well known. Generally, these color-forming compounds or couplers are colorless or substantially colorless. This lack of color is usually desirable where the coupler is to be incorporated in the emulsion layer and the unused coupler remains after formation of the colored image. When the coupler is used in the developing solution, it may be colored without detriment to the final image, and some colored couplers are known, such as paraphenylazo acetooacetanilide which was disclosed in Mannes and Godowsky Patent 2,108,602.

We have now found a new type of coupler which may have applications in several fields. The new couplers are, in themselves, more or less strongly colored, and during the coupling reaction, the chromophore system in the coupler is broken up with the result that the original color of the coupler is destroyed and a new dye is formed. Thus, on developing an emulsion layer containing one of these colored couplers, the coupler color is destroyed, and a new color is formed by the coupling reaction, at those points where development occurs. There is formed in this way a dye image of one color on a background of another color.

It is, therefore, an object of the present invention to provide a colored coupler whose chromophore system is destroyed on coupling. A further object is to provide a novel radical replacement type of chemical reaction. A still further object is to provide color couplers suitable for color correction processes of color photography. Other objects will appear from the following description of our invention.

These objects are accomplished by using as the coupler a phenolic compound having an azo group attached to the phenol nucleus in a position para to the hydroxyl group. These compounds have the following general formula:



where R is an aromatic or heterocyclic radical, especially an aromatic radical of the benzene series. Either the phenol nucleus or the aromatic or heterocyclic radical may contain other substituents. For example, the phenol radical may have a fused-on benzene ring which may be

5 further substituted. The aromatic or heterocyclic radical (R in the general formula) may contain substituents, such as alkyl, carboxylic acid, hydroxyl, sulfonic acid, sulfonamide, alkylamine, acylamine or alkoxy.

In previous descriptions of phenolic hydroxyl compounds for color photography, it has been assumed that the position para to the hydroxyl group must be unsubstituted or substituted with certain readily replaceable groups, such as halogen, in order for coupling with the developer to occur. We have found that the position para to the phenolic hydroxyl group may be substituted with an azo group and that this group is removable by the oxidized developer when the azo-substituted coupler is treated with the oxidized developer either in aqueous solution or in the photographic emulsion layer. Thus the coupler may be converted to a coupled compound and the azo group readily removed from it by means of reaction with the oxidized developing agent. This reaction appears to proceed as follows:



where R is the same as in the general formula above.

35 The following examples illustrate compounds which contain para-azo-substituted phenolic hydroxy groups according to the general formulas above and which may be used to produce colored images according to our invention:



X=H, OH, SO<sub>3</sub>H, SO<sub>2</sub>NH<sub>2</sub>, N(CH<sub>3</sub>)<sub>2</sub>, NHCOCH<sub>3</sub>, OCH<sub>3</sub>, COOH



3



Our compounds may be incorporated in the photographic developing solution or in the emulsion layer according to their intended use and diffusion characteristics. In the specific examples listed above, Nos. 4, 5, 6, and 8 are suitable for use in the emulsion layer. When incorporated in the emulsion layer, the compounds may be added directly to their silver halide emulsion as the sodium or other water-soluble salt or they may be incorporated in a coupler solvent as described in Mannes and Godowsky U. S. Patent 2,304,940 or Jelley and Vittum U. S. Patent 2,322,027.

The compounds employed according to our invention may be produced by any suitable method, such as by reaction of the phenolic compound with the appropriate diazonium compound. For example, compound No. 1 where X=COOH was prepared as follows:

4

Thirteen and seven-tenths grams (0.1 mole) of anthranilic acid were dissolved in a hot solution of 75 cc. of water and 30 cc. of concentrated hydrochloric acid. The solution was cooled to around 15° C. with stirring. Ice was then added and the mixture was diazotized by the addition of a solution of 7 g. (0.1 mole) of sodium nitrite in 25 cc. of water. More ice was added if necessary in order to keep the reaction temperature at 0 ± 3° C. After standing for ten minutes, the diazotized solution was added to a solution of 144 g. (0.1 mole) of α-naphthol in 100 cc. of water which contained 20 g. (0.5 mole) of sodium hydroxide. Ice was added in order to keep the temperature below 5° C. After standing for two hours at 5° C., the alkaline solution was acidified with 30 cc. of concentrated hydrochloric acid. The azo compound was removed by filtration, washed with water and dried in air. The yield was quantitative. After recrystallizing from acetic acid, the product melted at 239-240° C.

Our compounds are particularly useful in a process, such as that of Hanson U. S. Patent 2,449,966, granted September 21, 1948. The Hanson process involves a color correction method in which a colored coupler is incorporated in the photographic emulsion layer prior to exposure and upon development is converted into a colored image where the layer was exposed. The coupler remaining in the unexposed portions of the layer retains its original color, and by suitable choice of the color of the original coupler and the color of the final dye image, a masking or correction effect can be obtained.

Various photographic developing agents can be employed with the couplers of our invention. The primary aromatic amino developing agents are generally suitable including the phenylenediamines and aminophenols. The alkyl phenylenediamines may be substituted in the amino group as well as in the ring. Suitable compounds are diethylparaphenylenediamine, monomethyl para-phenylenediamine, dimethyl paraphenylenediamine and para-aminophenol. These compounds are usually employed in the salt form, such as the hydrochloride or the sulphate which are more stable than the free amines. All of these compounds have a primary amino group which enables the oxidation product of the developer to couple with the color-forming compounds to form dye images.

The following developing solution is suitable for developing gelatino silver halide layers containing colored couplers according to our invention.

|     |                                     |       |    |
|-----|-------------------------------------|-------|----|
| 55. | 2-amino-5-diethyl-amino toluene HCl | grams | 2  |
|     | Sodium sulphite                     | do    | 2  |
|     | Sodium carbonate                    | do    | 20 |
| 60. | Potassium bromide                   | do    | 2  |
|     | Water to                            | liter | 1  |

It will be understood that the examples and modifications set forth herein are illustrative only and that our invention is to be taken as limited only by the scope of the appended claims.

We claim:

1. The method of developing a colored image in a silver halide emulsion layer, which comprises incorporating in said layer a coupler compound having the formula:



where R is an aromatic nucleus selected from the class consisting of nuclei of the benzene and naphthalene series, said nucleus having the azo

group and the hydroxyl group para to each other, and R' is selected from the class consisting of aromatic and heterocyclic radicals, and said coupler compound contains no reactive phenolic hydroxyl group other than that to which the azo group is attached, exposing said layer and developing it with a primary aromatic amino developing agent, thereby splitting off the



group in said coupler compound and coupling said compound at the point of splitting with the oxidation product of the primary aromatic amino developing agent to form a dye image, leaving said coupler compound intact in the regions of said layer undeveloped by said developing agent.

2. The method of developing a colored image in a silver halide emulsion layer, which comprises incorporating in said layer a coupler compound having the formula:



where R is a naphthalene nucleus, said nucleus having the azo group and the hydroxyl para to each other, and R' is selected from the class consisting of aromatic and heterocyclic radicals, and said coupler compound contains no reactive phenolic hydroxyl group other than that to which the azo group is attached, exposing said layer and developing it with a primary aromatic amino developing agent, thereby splitting off the



group in said coupler compound and coupling said compound at the point of splitting with the oxidation product of the primary aromatic amino developing agent to form a dye image, leaving said coupler compound intact in the regions of said layer undeveloped by said developing agent.

3. The method of developing a colored image in a silver halide emulsion layer, which comprises incorporating in said layer a coupler compound having the formula:



where X is selected from the class consisting of hydrogen, hydroxyl, sulfonic acid, sulfonamido, dialkylamino, and acetylamino groups, and said coupler compound contains no reactive phenolic hydroxyl group other than that to which the azo group is attached, exposing said layer and developing it with a primary aromatic amino developing agent, thereby splitting off the



group in said coupler compound and coupling said compound at the point of splitting with the oxidation product of the primary aromatic amino developing agent to form a dye image, leaving said coupler compound intact in the regions of said layer undeveloped by said developing agent.

4. The method of developing a colored image in a silver halide emulsion layer, which comprises incorporating in said layer a coupler compound having the formula:



where R' is selected from class consisting of aromatic and heterocyclic radicals, and said coupler compound contains no reactive phenolic hydroxyl group other than that to which the azo group is attached, exposing said layer and developing it with a primary aromatic amino developing agent, thereby splitting off the  $-\text{N}=\text{N}-\text{R}'$  group in said coupler compound and coupling said compound at the point of splitting with the oxidation product of the primary aromatic amino developing agent to form a dye image, leaving said coupler compound intact in the regions of said layer undeveloped by said developing agent.

5. The method of developing a colored image in a silver halide emulsion layer, which comprises incorporating in said layer a coupler compound having the formula:



25 exposing said layer and developing it with a primary aromatic amino developing agent, thereby splitting off the



group in said coupler compound and coupling said compound at the point of splitting with the oxidation product of the primary aromatic amino developing agent to form a dye image, leaving said coupler compound intact in the regions of said layer undeveloped by said developing agent.

DUDLEY B. GLASS.

PAUL W. VITTMAN.

ARNOLD WEISSBERGER.

#### REFERENCES CITED

The following references are of record in the file of this patent:

#### 45 UNITED STATES PATENTS

|    | Number    | Name             | Date           |
|----|-----------|------------------|----------------|
| 50 | 1,102,028 | Fischer          | June 30, 1914  |
|    | 2,092,425 | Ullman et al.    | Sept. 7, 1937  |
|    | 2,107,941 | Hess et al.      | Feb. 8, 1938   |
|    | 2,108,602 | Mannes et al.    | Feb. 15, 1938  |
|    | 2,135,366 | Tinker           | Nov. 1, 1938   |
|    | 2,182,814 | Marasco          | Dec. 12, 1939  |
|    | 2,189,817 | Morris           | Feb. 13, 1940  |
|    | 2,220,123 | Schwarz          | Nov. 5, 1940   |
|    | 2,227,981 | Schinzel         | Jan. 7, 1941   |
|    | 2,263,012 | Schinzel         | Nov. 18, 1941  |
|    | 2,271,230 | Peterson et al.  | Jan. 27, 1942  |
|    | 2,295,008 | Porter et al.    | Sept. 8, 1942  |
|    | 2,295,009 | Porter et al.    | Sept. 8, 1942  |
|    | 2,297,732 | Woodward         | Oct. 6, 1942   |
|    | 2,299,641 | Middleton et al. | Oct. 20, 1942  |
|    | 2,304,820 | Hanford et al.   | Dec. 15, 1942  |
|    | 2,308,023 | Peterson         | Jan. 12, 1943  |
|    | 2,322,006 | Fierke et al.    | June 15, 1943  |
|    | 2,330,291 | Kirby            | Sept. 28, 1943 |
|    | 2,367,531 | Salminen         | Jan. 16, 1945  |

#### FOREIGN PATENTS

|    | Number  | Country       | Date          |
|----|---------|---------------|---------------|
| 70 | 503,752 | Great Britain | Apr. 11, 1939 |
|    | 503,824 | Great Britain | Apr. 11, 1939 |